

## 1

3,320,165

LUBRICANTS AND FUELS STABILIZED WITH  
ANTIOXIDANTS FOR HIGH AND LOW TEM-  
PERATURE CONDITIONS

Robert F. Bridger, Yardley, Leo J. McCabe, Princeton,  
and Albert L. Williams, Paulsboro, N.J., assignors to  
Mobil Oil Corporation, a corporation of New York  
No Drawing. Filed May 11, 1965, Ser. No. 454,993  
20 Claims. (Cl. 252—49.6)

This invention relates to the stabilization of lubricant and fuel compositions. Particularly this invention relates to additives providing protection against oxidation for such compositions over a broad temperature range.

Oxidation of lubricating oils takes place to a large extent in modern engines operated under normal conditions. The oxidation-deterioration products of oils, being acidic, can seriously corrode the metal surfaces of the engine. Moreover, a lubricant which has been subjected to oxidation cannot disperse the sludge readily, and permits the impurities to settle or become deposited inside the engine. As a result, the engine does not work efficiently.

Commercial lubricants, as well as fuels, are normally blended with agents known as antioxidants to prevent this deterioration. Unfortunately, many known antioxidants are only effective within a given temperature range. For example, if a low temperature antioxidant is subjected to heat at a high temperature it may be destroyed and the oil medium is susceptible to oxygen attack. On the other hand, although high temperature antioxidants can withstand heat longer, they may be ineffective at lower temperatures, and themselves destroyed. No fluid system in today's automotive or aircraft engines is operated at a constant temperature. A lubricating oil, for example, is continually subjected to high and low temperatures as it circulates through the lubricating system, e.g. from the sump to the engine block. For that reason antioxidant protection must be continuously available at both temperature levels. An oil passing over a high temperature surface must still be able to retain its low temperature antioxidant for protection in the subsequent cooler phase of the lubricating cycle. Conversely, the oil maintained temporarily at lower temperatures must retain its high temperature protection as it passes into the hotter stage. Moreover, this recirculation of oil from cold to hot regions on the system must last over a substantially extended period to be of any economical advantage. In the past, no effective engine lubricating system has been found in which the operating life of the antioxidant is sufficiently extensive.

It is therefore a major object of this invention to provide a novel combination of additives for lubricants and fuels. A further object is to provide an antioxidant composition for lubricants and fuels which is continuously operable at high and low temperatures. Another object of this invention is to provide antioxidants for lubricants and fuels which provide mutual protection for each other at high temperatures.

In accordance with this invention, it has now been discovered that lubricating oil and fuel compositions have extended antioxidant protection at varying temperature conditions by adding thereto in combination (1) a 9-hydroxy- or 9-alkoxy-9,10-boroxarophenanthrene and (2) an alkylated aromatic hydroxy compound having up to 7 aromatic rings or an aromatic secondary amine. Preferably

## 2

the aromatic hydroxy compounds are polyalkylated polyhydroxy phenols and polyalkylated naphthols.

The boroxarophenanthrene component is an extremely effective antioxidant at lower temperatures. Its properties 5 have been described in copending U.S. patent application Ser. No. 365,184, filed on May 5, 1964 (now patent 3,287,270). The general formula of these compounds is



wherein R may be hydrogen, alkyl, a term which includes also substituted alkyl, or alkenyl, cycloalkyl and haloalkyl having from 1 to about 25 carbon atoms. Suitable alkyl substituents for R may be methyl, tert.-butyl, dodecyl,  $\beta$ -methoxyethyl,  $\beta$ -aminoethyl, oleyl, 2-bicyclohexyl, and 1,1,7-trihydroperfluoroheptyl. The anhydride form of the compound may also be used, in which case R above is



R' and R'' may be alkyl, halogen or haloalkyl, and may be the same or different for each ring substitution and n is zero or an integer of 1 to 4, and preferably zero or 1 to 2.

The preparation of 9-hydroxy-9,10-boroxarophenanthrene, the preferred additive according to this invention, is achieved by the reaction of ortho-phenylphenol and boron trichloride; the product is heated in the presence of aluminum chloride to give 9-chloro-9,10-boroxarophenanthrene. The chloro compound is then hydrolyzed to the hydroxy. This procedure is described in detail in the above-mentioned application.

At temperatures of up to about 400° F., this compound is an exceptionally effective antioxidant for lubricating 50 oils. However, it becomes completely degraded in a very short time when exposed to temperatures above that level.

With respect to the second, or high temperature, component, this may be an alkylated aromatic hydroxy compound containing from 1 to 7 aromatic rings, such as a polyalkylated polyhydroxy phenol, a polyalkylated naphthol, or a secondary aromatic amine.

The polyalkylated polyhydroxy phenol has been disclosed as an antioxidant for lubricants in copending U.S. 60 Ser. No. 355,405, filed Mar. 27, 1964. These compounds include benzene, naphthalene and other aromatics, containing up to 7 rings either fused or connected by a single bond, as in biphenyl, or by an alkylene atom as in diphenylmethane. The alkyl substituents may have at least 65 4 carbon atoms attached to the nucleus, with at least 2

alkyl substitutions per compound. The preferred additives in this invention are the polyhydroxy benzenoid compounds having 2 to 3 hydroxy groups and 3 to 4 alkyl substituents with from about 12 to 30 carbon atoms.

An alternative second additive is the polyalkylated naphthol, disclosed in U.S. patent application Ser. No. 358,375, filed Apr. 8, 1964. These compounds include both alpha- and beta-naphthols having at least two alkyl substituents providing a total sum of alkyl carbon atoms of at least 8. Alkyl radicals having about 6 to about 30 carbon atoms are preferred.

A third class of high temperature antioxidants is a secondary aromatic amine having the formula



wherein  $\text{R}'''$  may be alkyl having from about 1 to about 25 carbon atoms, cycloalkyl, such as cyclohexyl, heterocyclic in which the cyclic structure has an oxygen, sulfur or second nitrogen atom, and aryl, such as phenyl or naphthyl, and substituted aryl, including such substituents as alkyl with from 1 to about 25 carbon atoms, halo, and haloalkyl, and Ar is an aromatic structure of 1 to 2 benzene rings, with up to five substituents including alkyl with from 1 to about 25 carbon atoms, halo, and haloalkyl; R and Ar may also be part of the same ring as in a heterocyclic structure. The secondary amines of this invention include N-phenyl-1-naphthyl amine, N-phenyl-2-naphthyl amine, diphenylamine, N,N'-diphenyl-p-phenylene diamine and the dimers thereof, and phenothiazine.

Specific preferred examples of the second component include tri-(2-hexadecyl)hydroquinone, tetra-(C<sub>15</sub>-C<sub>20</sub>-alkyl) resorcinol, tri-(2-hexadecyl)catechol, tris(2-hexadecyl) pyrogallol, tri-dodecyl-1-naphthol, 4,4-methylene-bis(2,6-di-tertiary-butyl-phenol), and the aforementioned N-phenyl-1-naphthyl amine.

We have discovered in this invention that the second component of these compositions, while performing as a high temperature antioxidant, e.g. at temperatures over 400° F., appears to prevent the heat from destroying the boroxarophenanthrene component. Were the first component to be used as the sole antioxidant for a fuel or lubricant composition, it would not function after exposure to high temperatures, e.g. near the engine block. The oil or other preponderant medium would deteriorate under oxidation. If the phenol, or the naphthol or the secondary amine were the sole component, the medium would be poorly protected against oxidation at temperatures below 400° F., in the sump or oil pan, for example, and the additive would be destroyed affording no protection to the oil as it later passes into the engine block. We have theorized that a mutual protection on the part of each additive, one for the other, has been manifested. Not only is the oil or fuel protected but also is the more susceptible additive under the temperature conditions at any instant.

Surprisingly, therefore, the compositions of this invention have longer high and low temperature service life than similar compositions using the components individually, even at higher concentrations. For example, the boroxarophenanthrene antioxidant is known to become deteriorated in several seconds at about 550° F.; in the instant compositions it may remain effective even after many hours of total exposure.

The quantity of the 9-hydroxy or 9-alkoxy-9,10-boroxarophenanthrene or derivative thereof which may be used is in the range of about 0.01% to about 25% by weight of the total composition; and preferably from about 0.01% to about 10% by weight for lubricants and from about 0.001% to about 5% by weight for fuels. The concentration of the high-temperature component is in the range of about 0.1% to about 25% by weight, and preferably about 0.5% to about 5%.

Discussion of the compositions of this invention have centered around lubricating oils and fuels in general; this is meant to include mineral oils, both solvent-refined and

acid-refined, hydrocarbon fuel fractions, polyolefins, dicarboxylic esters, trimethylol esters, pentaerythritol esters, polyalkylene oxides, phosphorus acid esters, silicones and the like. The compositions may therefore find utility not only as lubricants and fuels for automotive engines, but also as gear oils, turbine oils, aviation lubricants, transmission oils, hydraulic fluids, and marine oils. Moreover these formulations may also be combined with suitable thickeners, such as polyaromatic dye compounds or clays, to form oxidation-inhibited greases.

The following examples and tests are intended to illustrate more clearly the inventive concept without being a limitation on any aspect thereof.

#### PREPARATION OF 9-HYDROXY-9,10-BOROXAROPHENANTHRENE

Into a 1-liter flask were added 200 ml. of dry methylene chloride, held at -70° C. The flask was purged with nitrogen, and 235 grams (2.0 moles) of boron trichloride were bubbled in. To the contents were added dropwise, under agitation, 170 grams (1 mole) of o-phenylphenol in 200 ml. of methylene chloride, with the nitrogen atmosphere present. The temperature was maintained at -50° to -70° C. After the addition of the phenol, the reaction mass was stirred for 30 minutes at -70° C. and then was allowed to come to room temperature. Hydrogen chloride coming off was trapped in caustic solution. Stirring was continued for an additional hour and excess boron trichloride and methylene chloride were removed at 25° C. and 0.2 mm. Hg.

The brown liquid remaining was dissolved in 200 ml. of hexane and 5 grams of aluminum chloride were added, the mixture being held at 50° C. for 4 hours. Hydrogen chloride evolution ceased at this time. The product was filtered and the filtrate dissolved in 200 ml. of ether. The ether solution was shaken with 400 ml. of water in a separatory funnel. After the mixture was settled and the aqueous phase removed, the organic phase was concentrated under reduced pressure. A solid was formed, which was dissolved and recrystallized in benzene; M.P. 210-212° C. The ultra-violet spectrum analysis corresponded to the reported analysis of Deward and Dietz, J. Chem. Soc., London, 1960, pages 1344-1347.

*Analysis.*—Calc'd for C<sub>12</sub>H<sub>9</sub>O<sub>2</sub>B: B, 5.5%. Found: B, 5.9%.

The above product was tested in oil as the sole antioxidant and in combination with the aromatic amines and phenols in accordance with this invention.

#### DESCRIPTION OF TESTS

To simulate the conditions of the various parts of an engine lubricating system, the oil compositions are subjected to two tests successively at "high" and "low" temperatures. Control tests of fresh compositions are also run to better illustrate the unexpected nature of the invention.

*I. Thin-film oxidation test.*—In this test, the antioxidants are dissolved in a white oil (K.V. @ 210° F., 8 centistokes). The oil blend sample (140 ml.) is pumped through a preheater where it is heated to 550° to 600° F. and onto a heated aluminum disc contained in an enclosed chamber. The disc, held at 600° F., has a shallow conical face of 12 cm. in diameter and is rotated at 2500 r.p.m. The rotation causes the oil to spread into a thin film of about 0.0003 inch thickness over the disc surface. The approximate contact time of the oil on the disc is about 1 second. During the disc rotation, a stream of purified air is pumped continuously into the chamber at a constant rate of about 200 liters per hour. As the oil film becomes oxidized, the air that is consumed thereby is replaced automatically from a reservoir and the volume is recorded. The oil leaves the disc at the end of the one-second cycle and is cooled to 90° F. by means of a water jacket. Each sample is subjected to the test for 10 cycles.

II. *Low temperature oxidation test.*—Oxidation tests at a low temperature (302° F.) were conducted in an oxygen circulation apparatus of the type described by Dornte in Ind. Eng. Chem. 28, pages 26 to 30 (1936), modified to record the rate of oxygen absorption automatically. Broadly, in this test a tube containing the test oil sample is placed in a heater equipped with a thermostat control set at 302° F. After thermal equilibrium is established, the sample tube is connected with a closed oxygen circulating system. Oxygen is circulated through a fritted glass disc near the bottom of the sample tube at a rate of 5 liters per hour. The time required for the absorption of 50 millimoles of oxygen per 100 grams of sample is taken as the "induction period." The longer the induc-

5 Then the composition was diluted with 9 further portions of oil; in other words, the new concentration of the combined additives was reduced to  $\frac{1}{10}$  of its former level. This dilute composition was tested under the conditions of the low temperature oxidation test at 302° F., and the induction period was measured. A diluted composition was prepared as a control sample for each test sample and tested at 302° F. without the previous exposure in the thin-film test. Also reported are low temperature oxidation test results of  $\frac{1}{10}$  diluted oil compositions containing only the second additive without the boroxarophenanthrene compound. The results of these tests are tabulated in Table I; the term "BOP" refers to the boroxarophenanthrene compound.

10

TABLE I

| Example | Second Additive                                          | Weight percent <sup>1</sup> (Prior to thin film test) | Thin Film Test Temperature, °F. | 1/10-Diluted Composition Induction Period in 302° F. Low Temperature Test, Hrs. |                 |             | Theoretical percent of BOP Remaining |
|---------|----------------------------------------------------------|-------------------------------------------------------|---------------------------------|---------------------------------------------------------------------------------|-----------------|-------------|--------------------------------------|
|         |                                                          |                                                       |                                 | Pre-oxidized Oil                                                                | Control         | Without BOP |                                      |
| 1       | None                                                     |                                                       | 550                             | < 2 1                                                                           | 2 354           | -----       | 0                                    |
| 2       | Tri-(2-hexadecyl)hydroquinone                            | 2.74                                                  | 600                             | 92                                                                              | 79              | 5.7         | +100                                 |
| 3       | Tetra-(C <sub>15</sub> -C <sub>16</sub> alkyl)resorcinol | 3.74                                                  | 550                             | 81                                                                              | 69              | -----       | +100                                 |
| 4       | Tri-(2-hexadecyl)catechol                                | 2.71                                                  | 600                             | 10                                                                              | 36              | -----       | 28                                   |
| 5       | Tri-(2-hexadecyl)pyrogallol                              | 2.78                                                  | 600                             | 21                                                                              | 39              | -----       | 54                                   |
| 6       | 4,4'-methylenebis(3,6-di- <i>tert</i> -butylphenol)      | 2.75                                                  | 550                             | 151                                                                             | 180             | 41          | 84                                   |
| 7       | Tri-(dodecyl)-1-naphthol                                 | 2.25                                                  | 550                             | 80                                                                              | 100             | 19.2        | 80                                   |
| 8       | N-phenyl-1-naphthylamine                                 | 1.53                                                  | 550                             | <sup>2</sup> 39                                                                 | <sup>2</sup> 50 | 6.8         | 78                                   |

<sup>1</sup> Weight percentages are equivalent to about 0.035 mole per kg. of composition, except Example 6 (0.065 mole) and Example 3 (0.070 mole).

<sup>2</sup> The dilution of the 9-hydroxy-9,10-boroxarophenanthrene was 0.1% by weight (0.03% in the remaining tests).

<sup>3</sup> Test performed at 350° F.

tion period the greater is the oxidative resistance of the oil sample.

#### OXIDATION TEST RESULTS

##### Example I

A white oil was blended with 0.2% by weight of 9-hydroxy-9,10-boroxarophenanthrene. The oil solution was exposed to oxidation at 550° F. for only a single one-second cycle in the thin-film oxidation test. The resulting oxidized oil was then diluted with an equal amount of white oil (or about a 0.1% theoretical concentration of additive). This diluted blend was tested in the low temperature oxidation test. The induction period was less than one hour. A white oil containing no antioxidant also has an induction period of less than one hour in the low temperature test, indicating that the boroxarophenanthrene had been destroyed. Ultra-violet spectrum analysis confirmed the fact that the thin-film test lasting only one second at 550° F. completely destroyed the boroxarophenanthrene additive.

As a control, an oil blend containing 0.1% by weight of the 9-hydroxy-9,10-boroxarophenanthrene was tested in the low temperature test. The induction period was 354 hours.

##### Examples 2 to 8

Using the same white oil, compositions containing 0.3% by weight (0.0153 mole per kg. of composition) of 9-hydroxy-9,10-boroxarophenanthrene and varying amounts of the secondary additives disclosed in this invention were prepared. Each composition was first exposed to the thin-film oxidation for the full 10 cycles (a total of 10 seconds).

45 The results obtained from the above described tests indicate that the compositions of this invention have both high and low temperature antioxidant properties. The oil compositions could safely be operated in an engine lubricating system which subjects the oil to "hot" and "cool" regions successively.

50 Table I is indicative of the degree of protection given the boroxarophenanthrene compound at high temperatures. It also shows that the secondary compounds are equally susceptible at low temperatures. The following examples also indicate the protection afforded a representative group of these secondary additives by 9-hydroxy-9,10-boroxarophenanthrene.

##### Examples 9 to 12

60 A series of compositions of the white oil used in previous examples, containing 0.035 mole per kg. of composition of a phenol or naphthol alone was subjected to the low temperature oxidation test at 302° F. A second series of compositions, this time containing the phenol or naphthol plus 0.3% by weight (0.0153 mole per kg.) 65 of 9-hydroxy-9,10-boroxarophenanthrene, was also subjected to the same test, except that the test was continued 10 times as long as that of the corresponding composition in the first series.

70 Following each low temperature test, the compositions were subjected to the thin film oxidation test at the higher temperature. In the following table, the oxidation rate in the thin film test reflects the volume of oxygen absorbed. The lower the oxidation rate the better anti-oxidation is provided. The 9-hydroxy-9,10-boroxarophenanthrene is again herein referred to as BOP.

TABLE II

| Example | Antioxidants                                              | Weight Percent | Hours of Low Temperature Test at 302° F. | Temperature of Thin Film Test, F. | Oxidation Rate, ml. O <sub>2</sub> absorbed per 5 mins. |
|---------|-----------------------------------------------------------|----------------|------------------------------------------|-----------------------------------|---------------------------------------------------------|
| 9.      | None                                                      |                | 0                                        | 550                               | 440                                                     |
| 10.     | BOP                                                       | 0.30           | 0                                        | 550                               | 330                                                     |
| 10a.    | BOP                                                       | 0.30           | 45                                       | 550                               | 340                                                     |
| 11.     | Tri-(2-hexadecyl)hydroquinone                             | 2.74           | 0                                        | 600                               | 20                                                      |
| 11a.    | do                                                        | 2.74           | 12.7                                     |                                   |                                                         |
| 11b.    | { Plus BOP                                                | 2.74           | 127                                      | 600                               | 25                                                      |
| 12.     | Tetra-(C <sub>15</sub> -C <sub>21</sub> alkyl) resorcinol | 3.74           | 0                                        | 575                               | 20                                                      |
| 12a.    | do                                                        | 3.74           | 14.8                                     |                                   |                                                         |
| 12b.    | { Plus BOP                                                | 3.74           | 48                                       | 575                               | 20                                                      |
| 13.     | Tri-(hexadecyl)-catechol                                  | 2.71           | 0                                        | 600                               | 15                                                      |
| 13a.    | do                                                        | 2.71           | 14.5                                     |                                   |                                                         |
| 13b.    | { Plus BOP                                                | 2.71           | 145                                      | 600                               | 15                                                      |
| 14.     | Tri-(dodecyl)-1-naphthol                                  | 2.25           | 0                                        | 550                               | 15                                                      |
| 14a.    | do                                                        | 2.25           | 19.2                                     |                                   |                                                         |
| 14b.    | { Plus BOP                                                | 2.25           | 192                                      | 550                               | 15                                                      |

<sup>1</sup> Completely destroyed.

The data shown in Table II prove that the second additives alone cannot survive for more than several hours at the low temperatures and could then offer no oxidation protection at the high temperature level. However, the combination of the two additives furnishes protection which is greater than either of the two additives separately.

The combined 9-hydroxy or 9-alkoxy-9,10-boroxarophenanthrene and polyalkylated naphthol or polyhydroxy phenol or secondary aromatic amine may be used in the presence of other typical oil additives such as detergents, pour point depressors, viscosity control agents, and the like.

Although this invention has been described with the aid of specific embodiments and illustrations, the scope thereof is not limited thereby except as defined in the appended claims.

We claim:

1. A composition capable of withstanding oxidation at high and low temperatures successively comprising a major proportion of a member selected from the group consisting of mineral lubricating oils, synthetic lubricating oils, greases obtained therefrom and hydrocarbon fuels and a minor proportion, sufficient to provide antioxidant properties thereto, of (1) a boroxarophenanthrene of the formula



wherein R is selected from the group consisting of hydrogen, alkyl having from 1 to 25 carbon atoms and



R' and R'' are selected from the group consisting of alkyl, halogen, and haloalkyl, wherein the alkyl radicals have from 1 to 25 carbon atoms, and n is 0 to 4; and (2) an aromatic compound selected from the group consisting of a polyalkylated polyhydroxy hydrocarbyl aromatic

of an alkylated hydroxy hydrocarbyl aromatic compound having up to 7 ring nuclei and an aromatic secondary amine.

2. A lubricant composition capable of withstanding oxidation at high and low temperatures successively comprising a major proportion of a lubricating oil and a minor proportion, sufficient to provide antioxidant properties thereto, of (1) a boroxarophenanthrene of the formula



wherein R is selected from the group consisting of hydrogen, alkyl having from 1 to 25 carbon atoms, and



55 R' and R'' are selected from the group consisting of alkyl, halogen, and haloalkyl, wherein the alkyl radicals have from 1 to 25 carbon atoms, and n is 0 to 4; and (2) an aromatic compound selected from the group consisting of a polyalkylated polyhydroxy hydrocarbyl aromatic compound having up to 7 rings, a polyalkylated monohydroxy naphthol, and an aromatic secondary amine wherein at least one N-substituted group is an aromatic nucleus.

60 3. The composition of claim 2 wherein the R of the said boroxarophenanthrene is hydrogen.

4. The composition of claim 2, wherein the polyalkylated polyhydroxy hydrocarbyl aromatic compound is a phenol containing at least two hydroxy groups and the alkyl substituents having a total of at least 12 carbon atoms.

5. The composition of claim 2, wherein the polyalkylated monohydroxy naphthol contains at least two alkyl substituents having a total of at least 8 carbon atoms.

6. The composition of claim 2, wherein the secondary amine has the formula

Ar—N(H)—R'''

wherein Ar is an aromatic nucleus of 1 to 2 rings having up to 5 substituents selected from the group consisting of alkyl, halo, and haloalkyl, the alkyl group having 1 to 25 carbon atoms and R''' is selected from the group consisting of alkyl, cycloalkyl, haloalkyl, aryl, and alkaryl, wherein the alkyl groups have from 1 to 25 carbon atoms, and wherein Ar and R''' may also be members of a cyclic structure of which the amino nitrogen is a member.

7. A lubricant composition capable of withstanding oxidation at high and low temperatures successively comprising a major proportion of a lubricating oil and a minor proportion, sufficient to provide antioxidant properties thereto, of (1) a boroxarophenanthrene of the formula



wherein R is selected from the group consisting of hydrogen, alkyl having from 1 to 25 carbon atoms, and



R' and R'' are selected from the group consisting of alkyl, halogen, and haloalkyl wherein the alkyl radicals have from 1 to 25 carbon atoms, and n is 0 to 4; and (2) a polyalkylated polyhydroxy phenol having at least 2 hydroxy groups and at least 2 alkyl substituents, said alkyl substituents containing a total of at least 12 carbon atoms.

8. An oil composition capable of withstanding oxidation at high and low temperatures successively comprising a major proportion of a lubricating oil and a minor proportion, sufficient to provide antioxidant properties thereto, of (1) a boroxarophenanthrene of the formula



wherein R is selected from the group consisting of hydrogen, alkyl having from 1 to 25 carbon atoms, and



R' and R'' are selected from the group consisting of alkyl, halogen, and haloalkyl, wherein the alkyl radicals have

75

from 1 to 25 carbon atoms, and n is 0 to 4; and (2) a polyalkylated monohydroxy naphthol having at least 2 alkyl substituents containing a total of at least 8 carbon atoms.

5 9. An oil composition capable of withstanding oxidation at high and low temperatures successively comprising a major proportion of a lubricating oil and a minor proportion, sufficient to provide antioxidant properties thereto, of (1) a boroxarophenanthrene of the formula



wherein R is selected from the group consisting of hydrogen and alkyl having from 1 to 25 carbon atoms, and



25 35 R' and R'' are selected from the group consisting of alkyl, halogen, and haloalkyl, wherein the alkyl radicals have from 1 to 25 carbon atoms, and n is 0 to 4; and (2) an aromatic secondary amine of the formula

Ar—N(H)—R'''

40 40 wherein Ar and R''' are selected from the group consisting of aromatic radicals of 1 to 2 rings and members of a cyclic structure of which the amino nitrogen is also a member.

45 10. A lubricant composition capable of withstanding oxidation at high and low temperatures successively comprising a major proportion of a lubricating oil and a minor proportion, sufficient to provide antioxidant properties thereto, of (1) 9-hydroxy-9,10-boroxarophenanthrene and (2) an aromatic compound selected from the group consisting of a polyalkylated polyhydroxy phenol, the alkyl substituents having a total of at least 12 carbon atoms a polyalkylated monohydroxy naphthol having a total of at least 8 carbon atoms of the alkyl substituents, and an aromatic secondary amine of the formula

50 55 55 Ar—N(H)—R'''

wherein Ar and R''' are aromatic radicals having 1 to 2 rings and Ar and R''' may also be members of a cyclic structure of which the amino nitrogen is a member.

60 60 65 11. An oil composition capable of withstanding oxidation at high and low temperatures successively comprising a major proportion of a lubricating oil and a minor proportion, sufficient to provide antioxidant properties thereto, of (1) 9-hydroxy-9,10-boroxarophenanthrene and (2) a polyalkylated polyhydroxy phenol having 2 to 3 hydroxy groups and 3 to 4 alkyl radicals containing a total of at least 12 carbon atoms.

65 12. The oil composition of claim 11 wherein the said aromatic compound is tri-(2-hexadecyl)hydroquinone.

70 13. The oil composition of claim 11 wherein the said aromatic compound is tri-(2-hexadecyl)catechol.

14. The oil composition of claim 11 wherein the said aromatic compound is tri-(2-hexadecyl)pyrogallol.

15. The oil composition of claim 11 wherein the said aromatic compound is tetra-(C<sub>15</sub>—C<sub>20</sub> alkyl) resorcinol.

## 11

16. The oil composition of claim 11 wherein the said aromatic compound is 4,4'-methylenebis(2,6-di-tert.-butylphenol).

17. An oil composition capable of withstanding oxidation at high and low temperatures successively comprising (1) 9-hydroxy-9,10-boroxarophenanthrene and (2) a polyalkylated 1-naphthol containing from 6 to 30 carbon atoms per alkyl substituent.

18. The composition of claim 17 wherein the naphthol is tri-dodecyl-1-naphthol.

19. An oil composition capable of withstanding oxidation at high and low temperatures successively comprising a major proportion of a lubricating oil and a minor proportion sufficient to provide antioxidant properties thereto (1) 9-hydroxy-9,10-boroxarophenanthrene and (2) an aromatic secondary amine wherein the two carbons attached to the nitrogen are members of the group consisting of an aromatic ring and a cyclic structure of which the amino nitrogen is also a member.

## 12

20. The composition of claim 19 wherein the amine is N-phenyl-1-naphthyl amine.

## References Cited by the Examiner

## UNITED STATES PATENTS

|           |         |               |          |
|-----------|---------|---------------|----------|
| 2,009,480 | 7/1935  | Craig         | 252—50 X |
| 2,062,676 | 12/1936 | Reiff         | 252—50 X |
| 2,111,307 | 3/1938  | Bartram       | 252—50 X |
| 2,121,748 | 6/1938  | Suit          | 252—50 X |
| 2,191,499 | 2/1940  | Reiff         | 252—52 X |
| 2,672,448 | 3/1954  | Newman et al. | 252—52 X |
| 2,691,634 | 10/1954 | Benoit        | 252—52   |
| 3,211,652 | 10/1965 | Hinkamp       | 252—52   |

## FOREIGN PATENTS

565,012 10/1944 Great Britain.

DANIEL E. WYMAN, Primary Examiner.

W. H. CANNON, Assistant Examiner.